

## UNITED STATES PATENT OFFICE

2,472,627

FOG INHIBITOR FOR PHOTOGRAPHIC  
EMULSIONS

William F. Smith and Robert E. Stauffer, Rochester, N. Y., assignors to Eastman Kodak Company, Rochester, N. Y., a corporation of New Jersey

No Drawing. Application December 19, 1947,  
Serial No. 792,844

3 Claims. (Cl. 95—7)

1

This invention relates to fog-inhibiting agents and stabilizers for photographic emulsions and to photographic emulsions containing them.

It is known that photographic emulsions, particularly ultra-sensitive emulsions or those containing optical sensitizers exhibit a tendency to form upon development a deposit of silver in the emulsion. This deposit extends more or less uniformly over the entire emulsion and is known as fog. Photographic fog is of two types: local and general. Local fog is formed by exposure of the film or plate at undesired points as by a light leak in the camera. General fog is formed in a number of ways. It may be caused by the conditions under which the film or plate is stored, such as conditions of high temperature or humidity or unusually long time of storage. The nature of the emulsion may also produce general fog as well as the conditions of development of the emulsion as by development for protracted periods of time or at temperatures above normal. We are primarily concerned with fog and sensitivity changes produced in films or plates on development after storage under adverse conditions of high temperature and humidity or both.

General fog and loss of sensitivity of the emulsion are especially likely to occur when the sensitive material is stored under conditions other than ideal, that is, under conditions of high temperature and humidity as in tropical regions.

It is an object of the invention to provide novel anti-fogging or fog-inhibiting compounds for emulsions. A further object is to provide anti-fogging agents which stabilize the initial sensitivity of the emulsion. A still further object is to provide anti-fogging agents which improve the keeping of the emulsion in tropical regions. Other objects will appear from the following description of our invention.

These objects are accomplished by incorporating palladium nitrate into a silver halide emulsion.

The object of our invention is to maintain the sensitivity and fog of silver halide emulsions at or close to initial optimum values under keeping conditions of high temperature and humidity. The fog inhibitors which we propose to use are added to the emulsion during the process of manufacture to avoid loss of sensitivity and to inhibit the growth of incubation or keeping fog with pas-

age of time under non-ideal conditions of storage.

A solution of palladium nitrate,  $Pd(NO_3)_2$  when added in suitable concentration before coating to unsensitized or optically sensitized photographic emulsions does not affect appreciably the sensitometric values for sensitivity and fog when measurements are made soon after coating. When sensitometric measurements are made after appreciable intervals of time under tropical or dry conditions of storage at elevated temperatures, however, this compound does stabilize photographic speed and maintain fog at a low level.

The preparation of silver halide emulsions involves three separate operations, (1) the emulsification and digestion or ripening of the silver halide, (2) the freeing of the emulsion from excess soluble salts usually by washing, (3) the second digestion or after-ripening to obtain increased sensitivity (Mees, The Theory of the Photographic Process, 1942). We prefer to add the fog-inhibiting agents after the final digestion or after-ripening although they may be added before digestion. The most useful concentration range of fog inhibitor is from .260 to 3.90 gm. of fog inhibitor per kilogram of silver nitrate used in making the emulsion and converted to silver halide. This amount will vary, e. g. depending upon the particular silver halide used.

The anti-foggant and stabilizing action was determined by incubation of the emulsions under simulated tropical conditions and also by incubation in dry heat at 120° F. for various lengths of time after six days to one month. The results of these aging tests are tabulated here and are compared with the initial speed, gamma and fog of the emulsions with and without the anti-foggant and stabilizing compound. The tests from which the following tabulation was made used a high-speed orthochromatic negative type of emulsion exposed on an Eastman type IIB sensitometer and developed for five minutes in a developer of the following composition:

|                                   | Grams |
|-----------------------------------|-------|
| Monomethyl paraminophenol sulfate | 2.5   |
| Sodium sulfite (desiccated)       | 30    |
| Hydroquinone                      | 2.5   |
| Sodium Metaborate                 | 10    |
| Potassium bromide                 | 0.5   |
| Water to one liter                |       |

The results compared to other simple palladium salts are as follows:

scribed may be used in various kinds of photographic emulsions. In addition to being useful

| Sample No. | Gms. of compound per Kg. $\text{AgNO}_3$ (converted to $\text{AgX}$ ) in emulsion | Original   |       |     | 12 days 120° F. |       |     |
|------------|-----------------------------------------------------------------------------------|------------|-------|-----|-----------------|-------|-----|
|            |                                                                                   | 10/i Speed | Gamma | Fog | 10/i Speed      | Gamma | Fog |
| 1          | None                                                                              | 785        | 1.3   | .11 | 550             | 1.39  | .20 |
| 2          | $\text{Pd}(\text{NO}_3)_2$ , 1.03                                                 | 775        | 1.21  | .10 | 550             | 1.34  | .18 |
| 3          | $\text{Pd}(\text{NO}_3)_2$ , 1.55                                                 | 690        | 1.28  | .12 | 490             | 1.10  | .18 |
| 4          | $\text{Pd}(\text{NO}_3)_2$ , 2.06                                                 | 710        | 1.28  | .07 | 690             | 1.32  | .11 |
| 5          | $\text{PdSO}_4$ , 1.03                                                            | 210        | 1.48  | .14 | 110             | 1.59  | .29 |
| 6          | $\text{PdSO}_4$ , 1.55                                                            | 165        | 1.70  | .10 | 95.5            | 1.59  | .34 |
| 7          | $\text{PdSO}_4$ , 2.06                                                            | 55         | 1.78  | .32 | 57.5            | 1.59  | .27 |
| 8          | None                                                                              | 740        | 1.27  | .09 | 710             | 1.20  | .13 |
| 9          | $\text{PdCl}_2\text{H}_2\text{O}$ , 1.03                                          | 400        | 1.38  | .10 | 295             | 1.50  | .11 |
| 10         | $\text{PdCl}_2\text{H}_2\text{O}$ , 1.55                                          | 275        | 1.48  | .07 | 155             | 1.62  | .11 |
| 11         | $\text{PdCl}_2\text{H}_2\text{O}$ , 2.06                                          | 235        | 1.55  | .08 | 140             | 1.50  | .14 |

| Sam- ple No. | 18 days 120° F. |       |     | 4 weeks trop. |       |       | 8 weeks trop. |       |       |
|--------------|-----------------|-------|-----|---------------|-------|-------|---------------|-------|-------|
|              | 10/i Speed      | Gamma | Fog | 10/i Speed    | Gamma | Fog   | 10/i Speed    | Gamma | Fog   |
| 1            | 435             | 1.45  | .26 | 500           | 1.22  | .21   | 230           | 1.19  | .56   |
| 2            | 830             | 1.32  | .24 | 590           | 1.22  | .16   | 500           | 1.20  | .21   |
| 3            | 870             | 1.29  | .22 | 525           | 1.35  | .21   | 425           | 1.20  | .28   |
| 4            | 955             | 1.03  | .09 | 590           | 1.35  | .12   | 355           | 1.40  | .20   |
| 5            | 110             | 1.50  | .34 | black         | black | black | black         | black | >1.0  |
| 6            | 83              | 1.52  | .51 | black         | black | black | black         | black | >1.0  |
| 7            | 48              | 1.65  | .32 | 93.5          | 1.65  | .16   | 69.0          | 1.60  | .18   |
| 8            | 575             | 1.39  | .24 | 445           | 1.35  | .27   | 345           | 1.26  | .37   |
| 9            | 390             | 1.35  | .16 | black         | black | black | black         | black | black |
| 10           | 170             | 1.48  | .14 | black         | black | black | black         | black | black |
| 11           | 138             | 1.52  | .18 | black         | black | black | black         | black | black |

It will be noted from the data that the improvement in fog using the compound of the invention is appreciable as compared to the same tests carried out on the emulsion containing palladium sulfate or palladium chloride. In this respect, the compound of our invention is unique in that it represents one of the few simple salts of metals of the platinum group which are effective in reducing fog. In the Smith and Trivelli U. S. application Serial No. 792,843, filed concurrently herewith, now Patent No. 2,472,626, issued June 7, 1949, another simple salt of the platinum group, ruthenium tri-chloride, is described and claimed.

One of the advantages of our invention is the fact that the compound may be prepared with high purity compared to organic types of fog inhibitors. Another and perhaps chief advantage is the greater extent of stabilizing action over a wide range of climatic conditions.

In use, the fog inhibitor is dissolved in water at a convenient concentration and added to a melted gelatino-silver halide photographic emulsion in quantities ranging up to about 3.90 gms. per kilogram of silver nitrate converted to silver halide. The emulsion is coated on a suitable support, glass, film, or other, and dried in a normal fashion.

We also contemplate as a part of our invention those cases where it is desirable to coat the anti-foggant in a colloid layer such as gelatin on either or both sides of or also in the silver halide emulsion layer so that the anti-foggant is in at least one of the layers. In these cases, we use the same or a slightly greater ratio of rare metal salt to silver halide than when the salt is in the emulsion layer.

The fog-inhibiting agents which we have de-

35 in ordinary non-sensitized emulsions they may also be used in orthochromatic, panchromatic, and X-ray emulsions. If used with sensitizing dyes, they may be added to the emulsion before or after the dyes are added. Various silver salts may be used as the sensitive salt, such as silver bromide, silver iodide, silver chloride and mixtures of these. The dispersing agents may be 40 gelatin or other colloid such as collodion, albumen, cellulose derivatives, or synthetic resins.

It will be understood that we contemplate as 45 included within our invention all modifications and equivalents falling within the scope of the appended claims.

What we claim is:

1. A silver halide emulsion containing palladium nitrate.
2. A silver halide emulsion layer containing from 0.26 to 3.9 grams of palladium nitrate per kilogram of silver nitrate used in making said emulsion and converted to silver halide.
3. A light-sensitive photographic element comprising a silver halide emulsion layer and a colloid layer contiguous to said silver halide emulsion layer, at least one of said layers containing palladium nitrate.

WILLIAM F. SMITH.

ROBERT E. STAUFFER.

60

#### REFERENCES CITED

The following references are of record in the file of this patent:

65

#### UNITED STATES PATENTS

| Number  | Name                | Date           |
|---------|---------------------|----------------|
| 560,756 | Schoenfelder et al. | May 26, 1896   |
| 568,496 | Schoenfelder et al. | Sept. 29, 1896 |